

## UNITED STATES PATENT OFFICE

2,391,959

## SUN-BATHING APPAREL

George Gallowhur, Reading, Vt.

No Drawing. Application January 12, 1944.  
Serial No. 517,981

6 Claims. (Cl. 2—78)

This invention relates to sunbathing apparel; and more particularly to sunbathing apparel such as bathing suits, etc. which will permit the wearer thereof to acquire a uniform sun tan when exposed to the sun or other source of ultraviolet radiation.

The new sunbathing apparel of the present invention is made of thin, flexible, elastic, translucent thermoplastic sheets or films within which have been incorporated ultraviolet light filtering agents. Such apparel permits the pigmenting range of ultraviolet radiations to pass while effectively suppressing the erythema range, and enables the wearer of such apparel to derive the cosmetic and therapeutic benefits of exposure to sunlight or other sources of ultraviolet radiation without the heretofore attendant and objectionable inflammation.

The invention is of particular value in sunbathing apparel such as bathing suits and trunks which cover a considerable part of the body but which nevertheless permit the wearer thereof to acquire a uniform sun tan on the parts of the body so covered. The invention also includes other bathing apparel such as bathing caps, halters, trunks, shorts, sandals, slippers, belts, sunhats, bandannas, visors, etc. The apparel may also be in the form of garments or sheets which cover the entire body so that the entire body may be suntanned and at the same time protected from sunburn even after prolonged exposure to the sun or other ultraviolet radiation.

It is a common observation that the skin of a wearer of bathing apparel such as has heretofore been available does not tan uniformly when exposed to sunlight or another source of ultraviolet radiation. Those areas covered by the apparel remain substantially unaffected. Not only does this produce an undesirable cosmetic effect, but such lack of uniformity in pigmentation is believed to be biologically undesirable.

The present invention has as one of its objects to provide novel translucent sunbathing apparel which will effectively permit the passage of the desired range of ultraviolet radiation causing pigmentation (i. e., "tanning") and which will effectively suppress the passage of the undesirable range of ultraviolet radiation causing erythema (i. e., "sunburn"). Other objects of the invention will be apparent from the following description.

Since Dr. J. H. Kellogg first employed the sunbath systematically under medical supervision in 1876, heliotherapy has become a valuable adjunct in the prophylaxis and treatment of disease. The beneficial effects of ultraviolet radiation in the therapy of rickets were first noted by Huldschinsky, and it is established that certain wavelengths of this radiation caused a synthesis of antirachitic vitamin D from a precursor compound (ergosterol) in the skin (Laurens, *Physiol.* Rev.

8, 1 (1928)). Secondary anemia, various types of tuberculosis and certain skin infections are similarly amenable to heliotherapy. A deep-seated relation also exists between skin tanning and the sex hormone system in males (Hamilton and Hubert, *Science*, 88, 481 (1938)) and in females (Hamilton, *Proc. Soc. Exptl. Biol. Med.*, 40, 502 (1939)).

However, direct exposure to intense sunlight may have undesirable sequellae. Pigmentation (i. e., "tanning") is considered to have cosmetic value, but is often accompanied or preceded by an intense and painful erythema (i. e., "sunburn"). The relationship between pigmentation and erythema has been elucidated by Frydlander (Arch. *droguerie pharm.* 6, 4 (1938); *Chem. Zentr.* 1938 II, 1943; *Chem. Abst.* 34, 4863 (1940), and is important to an understanding of the present invention.

The ultraviolet spectrum covers the range of radiation between 136 and 4000 Angstroms. Part of this range, from 136 Å. to 1019 Å., is also considered as part of the X-ray spectrum. The shortest solar radiation that can reach the earth is about 2900 Å., so that the effective solar ultraviolet spectrum is from 2900 Å. to 4000 Å. The total amount of such radiation is never very great. On a clear day at sea level, the distribution of solar radiation is about 1-2% ultraviolet, 42-53% visible and 57-63% infrared. The limited therapeutic benefits derived from brief exposure to such radiation indicate the need for prophylactic measures, and the importance of adequate means for obtaining the range of radiation for optimum biochemical effect (Hawk and Bergelm—Practical Physiological Chemistry, X edition, pg. 663).

The radiation causing erythema is in the region of 2967 Å. Radiations of 3261 Å. cause only 0.3% to 0.4% of the inflammation resulting from an equivalent exposure of 2967 Å. radiations, although the pigment formation (i. e., "tanning") at 3261 Å. is considerable.

The new sunbathing apparel of the present invention has incorporated therein ultraviolet light filtering agents and particularly agents protecting the skin from radiations between 2950 Å. and 3100 Å., such that the apparel will permit tanning without sunburn. These agents are incorporated in the thin, flexible, elastic, translucent thermoplastic sheets or films of which the apparel is made.

In general, the protective agents used in the thin translucent film material of which the apparel is made include those which have the specific ability to suppress radiation of 2967 Å., such substances being effective ultraviolet light filters for protection against sunburn. Certain agents such as certain fluorescent compounds do not absorb the ultraviolet radiation completely but

rather convert such radiation into other wavelengths which do not cause erythema.

A typical example of such an ultraviolet light filter for use in making the new apparel is beta-methyl umbelliferone (Parfumerie Moderne, May, 1936, pp. 203-209). The percent transmission by a 1% solution of beta-methyl umbelliferone of ultraviolet radiations of different wavelengths is as follows:

|        | Per cent | Per cent |       |
|--------|----------|----------|-------|
| 2894 Å | 3.0      | 3129 Å   | 0.03  |
| 2967 Å | 0.6      | 3341 Å   | 0.40  |
| 3021 Å | 0.02     | 3650 Å   | 94.00 |

Thus, it can be seen that the "erythema range" of ultraviolet radiations, 2950 Å-3100 Å, can be effectively screened out although longer and shorter wavelengths of ultraviolet light will pass the filter.

In making the new sunbathing apparel there is first made a thin, flexible, elastic, translucent, thermoplastic sheet or film within which has been incorporated the ultraviolet, light filtering agents, and such sheets or films are then used in making the new sunbathing apparel.

The term "translucent" as used in the specification and claims, refers to those opaque plastics which in thin sheet or film form permit the passage of substantially the entire range of ultraviolet radiations. For the products of the present invention, i. e., sunbathing apparel, the use of the transparent plastics is obviously unfeasible, and plastics are used which in thin sheet or film form possess the property of opacity to visible radiations, while nevertheless permitting passage of the pigmenting range of ultra-violet radiation.

When the thin, flexible, elastic, translucent thermoplastic films have suitable ultraviolet light filtering agents incorporated therein, such apparel permits the pigmenting range of ultraviolet radiations to pass while effectively suppressing the erythema range, and the wearer of such apparel may derive the cosmetic and therapeutic benefits of exposure to sunlight or other sources of ultraviolet radiation without attendant and objectionable inflammation.

Typical members of the group of materials which can be used as thermoplastics are regenerated cellulose, cellulose ester and cellulose ether sheeting (e. g., Lumarith, Tenite, Plastacele), rubber hydrochloride (e. g., Parlon, Pilofilm) and some types of long-chain polyamides (nylon). The more typical members of this group and those more readily applicable to the products of the present invention, are the so-called "vinyl resins." A good definition of this term is given by Akin (Chemical Industries, LII, 456, April, 1943):

"Commonly, the term 'vinyl resins' is taken to mean polymers or co-polymers of vinyl esters and ethers as typified by the following structures, or products derived by subsequent condensations based on such resins:

|                                       |                     |
|---------------------------------------|---------------------|
| $\text{CH}_2:\text{CHCl}$             | Vinyl chloride      |
| $\text{CH}_2:\text{CHOH}$             | Vinyl alcohol       |
| $\text{CH}_2:\text{CCl}_3$            | Vinylidene chloride |
| $\text{CH}_2:\text{CHOCOCH}_3$        | Vinyl acetate       |
| $\text{CH}_2:\text{CHOC}_2\text{H}_5$ | Vinyl ethyl ether"  |

Typical vinyl resins available industrially are the following:

Vinyl chloride polymers—Flamenol, Korogel, Korolac, Koroseal, Vinylite Q.

Vinyl acetate polymers—Gelva, PV Acetate, Vinylite A

Vinyl chloride-vinyl acetate copolymers—Tygon, Vinylite V, Vinyon, Vinylseal

Vinylidene chloride polymers—Apla, Saran, Velon

Vinyl alcohol polymers—PVA, Solvar

Vinyl ethyl ether polymers—Lutonal

Condensation products of polymerized vinyl alcohol—

With formaldehyde—Formex, Formvar

With acetaldehyde—Alvar

With butyraldehyde—Butacite, Butvar, Flex-seal, Heydenite, Safex, Vinal, Vinylite X

With benzaldehyde—Benvar

With crotonaldehyde—Crotvar.

The term "ultraviolet light filtering agents" as used in the specification and claims of the present invention refers to those compounds capable of absorbing at least the erythema range of ultraviolet radiations, i. e., 2950 Å. to 3100 Å., and converting them to radiations of either shorter or longer wavelengths than that range. These compounds bear no common chemical resemblance to each other but are characterized by this sole physical property of re-emission of absorbed ultraviolet light. When this re-emitted light is visible, the phenomenon is called fluorescence.

Typical "ultraviolet light filtering agents" applicable in the products of the present invention are: beta-methyl umbelliferone, glyceryl p-aminobenzoate, menthyl salicylate, glyceryl salicylate, glycol salicylate, quinine bisulfate and other quinine and cinchona alkaloid salts, hexahydroxyethyltannic acid, esculin, esculetin, stilbene, sodium 2-phenylbenzimidazole-5-sulfonate, 2-phenylbenzoxazole, menthyl anthranilate, cyclohexenylanthranilate, isosafrole, benzalacetophenone, dibenzalacetone, 9-ethyl,3-dimethylaminocarbazole, 4-methyl,7-diethylaminocoumarin, 3-methyl,5-dimethylaminoazimidobenzene, 2-(p-aminophenyl)5-aminobenzimidazole, 2-phenyl,5-aminobenzoxazole, 3-dimethylaminoacridine, alkyl 3-methoxy-o-coumarate, triethanolamine o-cresotinate, triethanolamine 2,3-hydroxynaphthoate, dibenzalazine, hydroquinone, chlorophyll derivatives such as pheophytin, pheophorbide, phytochlorine and photorhodine, 2-hydroxybenzalacetoneoxalate esters, 2-chlorbenzalacetoneoxalate esters, furfuralacetoneoxalate esters, cinnamalacetoneoxalate esters, and many other compounds. In general, any non-toxic compound can be used as an ultraviolet light filtering agent that is compatible with the chemical nature of the thermoplastic, and that will absorb at least the range of ultraviolet radiations from 2950 Å. to 3100 Å. and entirely suppress this range and/or re-emit it as radiations of smaller or greater wavelengths. A large number of such compounds are listed and discussed in De Ment's "Fluorescent Chemicals and Their Applications" (Chemical Publishing Co., 1942). These compounds may be organic, inorganic, or metallo-organic in nature.

The thermoplastic materials used in making the flexible, elastic, translucent films of which the sunbathing apparel is made are suitably compounded according to various processes available in the compounding art. With some materials the compounding may be effected in a solution of the material from which the flexible, elastic, translucent film is obtained by evaporation of the solvent. With thermoplastic resins the com-

pounding will in general be effected by fluxing in a heated mixer with the addition of the requisite plasticizers, opacifiers, dyes or pigments, lubricants and stabilizers. Into this mixture may now be incorporated the requisite amount of the ultraviolet light filtering agent. This amount may vary from traces, to 20% of the total weight of the composition, depending on the chemical nature of the filtering agent. This filtering agent may also serve additional or ancillary purposes. It may replace all or part of the plasticizing agent. When present in an amount in excess of its solubility in the composition, it may serve as an opacifying agent. It may also serve as a lubricant and as a stabilizing agent.

The hot resin "dough" is then mixed further in an ordinary rubber mill to obtain better dispersion of the ingredients, and is then calendered into sheeting (material thicker than 0.005 inch) or film (material 0.005 inch thick, or less). Thickness usually runs in standard gauges e. g., 0.004, 0.008, 0.020, 0.040 and 0.085 inch. In general, if the original resin has an average molecular weight between 15,000 and 22,000, the resultant plastic forms a translucent, resilient, elastic sheet that is tough, strong, durable and washable. Such sheets are well suited for use in making the apparel of the present invention.

Other methods of incorporating the ultraviolet light filtering agent than those above described may be used. Thus, the agent may be mixed with the monomer of the plastic and the latter is then polymerized (or co-polymerized, if a mixture of monomers is present). The filtering agent will thus become an integral part of the finished plastic. Alternatively, a sheet of the ultraviolet light filtering agent may be bonded between two sheets of the translucent or transparent plastic.

In general, the present invention involves the construction of sunbathing apparel of elastic, translucent thermoplastics containing ultraviolet light filtering agents as integral components thereof, irrespective of the manner in which said filtering agents have been incorporated.

Such sheets or films of plastic material containing the ultraviolet light filtering agent are used in making the new sunbathing apparel of the present invention. The garments such as bathing suits may be made by cutting the thin, flexible, elastic, translucent films or sheets into suitable pieces or patterns and combining these to make the garments. The material can be shaped, pressed, embossed, sewed or cemented and in some cases may be heat-sealed, depending upon the particular plastic material used. The cut film when shaped and suitably combined by sewing, cementing, or heat-sealing, etc., forms the garment or other sunbathing apparel. Such garments being made of thin, flexible and elastic material and properly shaped and made, are pleasing in appearance, and can be worn with much the same facility and comfort as ordinary bathing suits and similar apparel.

The new bathing suits and other sunbathing apparel of the present invention may be made in different colors and patterns. Although translucent in the sense hereinbefore described such that they permit the passage of the pigmenting range of ultraviolet radiations to pass while effectively suppressing the erythema range, they are opaque to visible radiations.

The thin, flexible, elastic, translucent plastic sheets or films used in making the new sunbathing apparel can also be used in sheet form for covering the body while being exposed to sunlight

5 or other ultraviolet radiation to protect the body from sunburn while permitting the desirable and beneficial effects of such exposure. When the body is so covered and protected it may be subjected to prolonged exposure to sunlight or other ultraviolet radiation without objectionable sunburn.

10 It will thus be seen that the present invention provides sunbathing apparel which while protecting the wearer and being opaque in appearance is nevertheless translucent and permits a desirable transmission of the pigmenting range of ultraviolet radiation to permit tanning of the parts of the body covered by the apparel while nevertheless protecting such parts of the body from sunburn.

I claim:

1. Sunbathing apparel made of thin, flexible, translucent, thermoplastic sheets containing ultraviolet light filtering agents, said apparel being opaque to visible radiations and permitting the pigmenting range of ultraviolet radiations to pass while effectively suppressing the erythema range, and enabling the wearer of the apparel to acquire a suntan without sunburn on the parts of the body covered by the apparel.

2. Sunbathing apparel made of thin, flexible, elastic, translucent, thermoplastic sheets containing agents to prevent the passage of at least the 2950 Å. to 3100 Å. range of ultraviolet radiations, said apparel being opaque to visible radiations and permitting the pigmenting range of ultraviolet radiations to pass while effectively suppressing the erythema range, and enabling the wearer of the apparel to acquire a suntan without sunburn on the parts of the body covered by the apparel.

3. Sunbathing apparel made of thin, flexible, translucent, vinyl resin thermoplastic sheets containing ultraviolet light filtering agents, said apparel being opaque to visible radiations and permitting the pigmenting range of ultraviolet radiations to pass while effectively suppressing the erythema range, and enabling the wearer of the apparel to acquire a suntan without sunburn on the parts of the body covered by the apparel.

4. Sunbathing apparel made of thin, flexible elastic, translucent, vinyl resin thermoplastic sheets containing agents to prevent the passage of at least the 2950 Å. to 3100 Å. range of ultraviolet radiations, said apparel being opaque to visible radiations and permitting the pigmenting range of ultraviolet radiations to pass while effectively suppressing the erythema range, and enabling the wearer of the apparel to acquire a suntan without sunburn on the parts of the body covered by the apparel.

5. Sunbathing apparel made of thin sheets of at least one member of the group of flexible, elastic, translucent, vinyl resin thermoplastics consisting of vinyl chloride polymers, vinyl acetate polymers, vinyl chloride and vinyl acetate copolymers, vinyl alcohol polymers, vinylidene chloride polymers, and their condensation products with aliphatic and aromatic aldehydes, containing ultraviolet light filtering agents, said apparel being opaque to visible radiations and permitting the pigmenting range of ultraviolet radiations to pass while effectively suppressing the erythema range, and enabling the wearer of the apparel to acquire a suntan without sunburn on the parts of the body covered by the apparel.

6. Sunbathing apparel made of thin sheets of at least one member of the group of flexible,

translucent vinyl resin thermoplastics consisting of vinyl chloride polymers, vinyl acetate polymers, vinyl chloride and vinyl acetate copolymers, vinyl alcohol polymers, vinylidene chloride polymers, and their condensation products with aliphatic and aromatic aldehydes, containing agents to prevent the passage of at least the 2950 Å. to 3100 Å. ranges of ultraviolet radiations, said apparel be-

ing opaque to visible radiations and permitting the pigmenting range of ultraviolet radiations to pass while effectively suppressing the erythema range, and enabling the wearer of the apparel to acquire a suntan without sunburn on the parts of the body covered by the apparel.

GEORGE GALLOWHUR.